

# UNITED STATES PATENT OFFICE.

HANS GOLDSCHMIDT AND OTTO WEIL, OF ESSEN-ON-THE-RUHR, GERMANY, ASSIGNORS TO  
THE FIRM OF TH. GOLDSCHMIDT, OF ESSEN-ON-THE-RUHR, GERMANY.

## METHOD OF MANUFACTURING METALS.

No. 895,628.

Specification of Letters Patent.

Patented Aug. 11, 1908.

Application filed October 9, 1905. Serial No. 282,050.

*To all whom it may concern:*

Be it known that we, HANS GOLDSCHMIDT and OTTO WEIL, both subjects of the King of Prussia, German Emperor, and residents of 5 Essen-on-the-Ruhr, in the German Empire, have jointly invented a new and Improved Method of Manufacturing Metals, of which the following is an exact specification.

Our invention relates to a new and improved method of manufacturing metals as hitherto made according to the well-known alumino-thermic or so-called "Goldschmidt"-process and for producing such metals we start with the metallic oxids such as oxid 15 of chromium for the purpose of producing chromium. The metal thus produced has found a wide range of use in the steel manufacture and large quantities of same are wanted there, for the advantages of using 20 such metals free from carbon have been tested and generally acknowledged. As the price of the metal is high it is naturally a desideratum to cheapen the process of production.

25 Now it is the object of our invention to make the above mentioned Goldschmidt-process a more economical one or in other words to increase the output of metal over the one produced in the Goldschmidt-process 30 but without increasing the quantities of chromium oxid used.

In the Goldschmidt process an oxid of chromium  $\text{Cr}_2\text{O}_3$  is employed, which represents the lowest degree of oxidation applicable for practical purposes. Now it has been found, that by using  $\text{Cr}_2\text{O}_3$  a comparatively small output of metal is gained, which result is due to the slow proceeding of the reaction taking place, so that but little metal 40 separates. If however, chromium of a higher degree of oxidation is used, the reaction sets in too quickly, its course is a rather turbulent one and involves danger as well as loss of metal. The employment of our 45 method as described herein avoids these defects and increases the output of metal by about 30-40%.

The most important novelty of our new method is the fact discovered by us, that but 50 a comparatively small quantity of metallic oxid of a higher degree of oxidation will suffice as addition to the well known Goldschmidt mixture to bring about the desired result, for example 1% of chromic acid added to oxid of chromium. This additional

small percentage of oxid of high degree of oxidation serves as a stimulant for a faster reaction to take place and at the same time it causes the formation of an easily melting slag, whereas the usual chrome slag is known 60 to have a high melting power.

In carrying out our process in practice it is of considerable advantage, if the slag is prevented from becoming rigid too soon, as this result assists a good deal in gaining a fine 65 regulus of chromium.

Thus the feature of our invention consists in the mixture of a small quantity of a metallic oxid of a high degree of oxidation with a large quantity of metallic oxid of a low degree of oxidation, of which mixture the oxid of higher degree serves the purpose of quickening the pace of the reaction and the oxid of lower degree acts as a safeguard against dangerous effects and destruction of metal 70 during this reaction.

We shall now attempt to show by way of example, how the process of manufacturing chromium is carried out according to our method; 100 kilos of pure oxid of chromium 80 are thoroughly mixed with 3-4 kilos of chromic acid, to which mixture 34-35 kilos of aluminium of finest granulation are added. The reaction is then started in this mixture by igniting at a point in the manner well understood in the above mentioned Goldschmidt process. In this composition the particles of chromic acid evenly distributed 85 in the whole mixture, serve as an agent for initiating and transmitting the reaction to 90 all parts of the mass.

We claim:

1. Method of manufacturing metals according to the alumino-thermic process consisting in mixing an oxid of the metal concerned with another oxid of the same metal of higher oxidation and adding thereto finely granulated aluminium, then igniting the mixture in order to start the reaction.

2. Method of manufacturing metals according to the alumino-thermic process consisting in mixing an oxid of the metal concerned of low oxidation with a very small percentage of an oxid of the said metal of higher oxidation and adding thereto finely 100 granulated aluminium, then igniting the mixture in order to start the reaction.

3. Method of manufacturing chromium consisting in mixing a small percentage of chromic acid with chromium oxid ( $\text{Cr}_2\text{O}_3$ ) 110

adding thereto finely granulated aluminium and then starting the reaction by igniting.

4. Method of manufacturing chromium consisting in mixing 3 parts of chromic acid with 100 parts of oxid of chromium ( $Cr_2O_3$ ), adding thereto 34 parts of finely granulated aluminium and then starting the reaction by igniting the mixture.

In witness whereof we have hereunto set our hands in the presence of two witnesses. 10

HANS GOLDSCHMIDT.  
OTTO WEIL.

Witnesses:

WILLIAM ESSENWEIN,  
RUDZ LIEBER.